

# UNITED STATES PATENT OFFICE.

JAMES E. SHEAFFER, OF BURNHAM, PENNSYLVANIA.

## COMPOUND FOR COVERING THE TOP OF MOLTEN METAL IN INGOT-MOLDS.

1,212,825.

Specification of Letters Patent.

Patented Jan. 16, 1917.

No Drawing.

Application filed April 20, 1916. Serial No. 92,514.

To all whom it may concern:

Be it known that I, JAMES E. SHEAFFER, a citizen of the United States, and a resident of Burnham, county of Mifflin, State of Pennsylvania, have invented certain Improvements in Compounds for Covering the Top of Molten Metal in Ingot-Molds, of which the following is a specification.

The object of my invention is to prevent, as much as possible, the formation of piping in ingots during the casting operation. This object I attain by placing on the top of the molten metal, after it has been poured in the ingot, a suitable composition which will retain the heat in the upper portion of the ingot until the major portion of the ingot commences to cool, when the entire mass will cool evenly, thus materially reducing the depth of the piping in the upper end of the ingot.

Heretofore, it has been the practice to place a layer of plumbago on the top of the molten metal so as to reduce the depth of the piping, but this material is now very expensive and I find that by the use of the compound which I will proceed to describe, good results can be attained with a great reduction in cost.

The compound which I use is a mixture of pulverized anthracite coal mixed with a petroleum oil, the oil being in such proportion as to make a plastic mass which is placed on top of the molten steel immediately after it has been poured in the ingot molds. Owing to the fact that all anthracite coal has a tendency to coke together during combustion and form clinker, the coal alone cannot be successfully used to protect the surface of the molten steel in the ingot mold, because instead of following the contour of the steel as it cools, the coal during its com-

bustion exercises this tendency to clinker and thereby bridges over the space, holding the protecting coal away from the steel at one or more points. By the addition of petroleum oil, I overcome this tendency to bridge so that the protecting compound will follow the contour of the steel as it cools and will thus be an efficient protective covering.

The mixture I have used with success is one quart of petroleum oil to one hundred pounds of carbonaceous material, but it will be understood that the proportions of the ingredients may be varied without departing from the essential features of the invention.

While I have used a petroleum oil, other hydrocarbons may be used, such as paraffin, without departing from the spirit of the invention.

I claim:

1. A compound for protecting the exposed surface of molten steel in an ingot mold, said compound consisting of a mixture of pulverized coal with a hydrocarbon, the coal being in excess, and the hydrocarbon preventing the coal from bridging over the steel in the ingot mold as it cools.

2. A compound for protecting the exposed surface of molten steel in an ingot mold, said compound consisting of a mixture of pulverized anthracite coal and petroleum oil, the anthracite coal being in excess.

3. A compound for protecting the exposed surface of molten steel while in an ingot mold, said compound consisting of a mixture of pulverized anthracite coal and petroleum oil in about the proportion of one quart of petroleum to one hundred pounds of anthracite coal.

JAMES E. SHEAFFER.